

## UNITED STATES PATENT OFFICE

2,231,891

PROCESS OF PRODUCING NATURAL OR  
ARTIFICIAL FIBERS HAVING DYEING  
PROPERTIES RESEMBLING THOSE OF  
WOOL AND PRODUCTS OBTAINED THERE-  
BYPaul Esselmann, Wolfen, Kreis Bitterfeld, and  
Josef Dusing, Dessau, Germany, assignors, by  
mesne assignments, to Walther H. Duisberg,  
New York, N. Y.No Drawing. Application December 7, 1938, Se-  
rial No. 244,388. In Germany August 4, 1937

5 Claims. (Cl. 8—113)

Our present invention relates to the production of fibers, foils, threads, ribbons and the like materials which are capable of being dyed with acid wool dyestuffs.

5 We have previously disclosed in our application Ser. No. 223,012, filed August 4, 1938, that it is possible to produce artificial textile materials capable of being dyed with acid wool dyestuffs in the same manner as wool by incorporating 10 and finely dispersing in the solutions from which the textile materials are to be formed a synthetic resinous composition stable against dilute acids and alkalies which resinous composition is the product of the joint polymerization of an 15 alkylene imine and a protein and an arylisocyanate or an arylisothiocyanate.

By the present application which is a continuation in part of the aforesaid application Ser. No. 223,012 we extend the application of 20 the said resinous compositions also to natural cellulosic fibers and to artificial fibers in such cases where it is not desirable or possible to introduce or finely disperse the resinous compositions in the spinning solutions.

25 The present invention therefore has for an object to provide textile materials such as threads, fibers, foils, ribbons and the like which may be easily dyed with acid wool dyestuffs.

A still further object resides in the provision 30 of fibers which are impregnated with basic reacting resins and which are capable of being dyed directly with acid wool dyestuffs.

Additional objects will appear from the following detailed specification.

35 We have found that by impregnating artificial fibers or natural fibers such as for instance cotton with an alkylene imine or a similar organic base, a solution of an albuminous substance, a solution of an arylisocyanate or an arylisothiocyanate and heating the impregnated fibers to a temperature sufficiently elevated to cause polymerization of the alkylene imine with the isocyanate, fibers are obtained which have exactly the character of wool as regards the capacity of being dyed with acid dyes and the fastness of the 40 dyeings to washing and to light. We are aware that processes of impregnating fibers with various substances including resins have been proposed. The dyeings on the fibers hitherto produced according to these processes have been unable to satisfy practical requirements as regards properties of fastness in all respects. Contrary to these prior art proposals the present invention provides fibers which are characterized 45 by sufficient fastness to washing, perspiration,

rubbing and other friction, and satisfactory fastness to light.

Fibers which have been made from casein solutions of course do not need an additional impregnation with an albuminous substance. In 5 these cases it is sufficient to impregnate the artificial fibers with alkylene imines and the aromatic isocyanate. After the impregnation the resin may be produced on the fibers by polymerization which can be effected by heating. The 10 dyeings with wool dyestuffs on casein fibers in this manner are essentially faster than dyeings on ordinary casein fibers which have not been impregnated with the resins.

The fibers may be impregnated with the finished resinous compositions in solution whereafter further condensation on the fibers is effected by a short additional heating. On the other hand they may be impregnated with the constituents of the resin and condensation may 20 be effected on the fibers by heating and drying.

Suitable starting materials for the polymerization have been described in our copending U. S. patent application Ser. No. 223,013 filed 25 August 4, 1938.

The following may be mentioned as examples.

Suitable organic bases are, for instance, the alkyleneimines, such as ethylene-, propylene- and butylene-imines, N-propyl-ethyleneimine and N-benzylethyleneimine.

Furthermore aliphatic and aromatic amines, such as methylamine, stearylamine and aniline may be employed.

Suitable protein substances are casein, albumen, gelatin, and the like materials.

As aryliso- and arylisothiocyanates there may be employed mainly the phenyl- and naphthyl-isocyanates as well as the phenyl- and naphthyl-isothiocyanates, benzylisocyanate, and related 40 compounds.

The following examples serve to illustrate the invention.

## Example 1

Fibers made from casein or fibers containing 45 casein are immersed in a benzene solution of 30 per cent strength of ethyleneimine and led through the solution several times by means of creasing rollers. After the ethyleneimine solution has acted upon the fibers for about 30 minutes the adhering liquid is removed from the fibers, if necessary by centrifuging, and they are immersed in a solution of phenylisocyanate for a few minutes. The fibers are then removed from the phenylisocyanate solution. Thereupon they 50

55

are thoroughly centrifuged, steamed for some time and then dried. After drying the fibers are advantageously washed once more in soap water.

5

*Example 2*

A strand of cotton is immersed in a solution of 1 part of casein, 5 parts of an aqueous ethylene-imine solution of 30 per cent strength and 5 parts of phenylisocyanate. The impregnated cotton threads are centrifuged and heated for an hour at a temperature of 7° C. A polymerization product is formed on and in the cotton fibers which adheres strongly thereto and cannot be removed by scouring and washing. The cotton fibers acquire a distinct affinity for acid dyestuffs such as for instance Palatine Fast Blue BR (Schultz Farbstofftabellen, vol II, 7th edition, page 168), Supramine Red B (Schultz Farbstofftabellen, vol. II, 7th edition, page 203), Acid Antracene Red 3 BL (Schultz Farbstofftabellen, Suppl. vol. I, 7th edition, page 125) and metachrome dyestuffs. The dyeings on these fibers are absolutely fast to light.

25

*Example 3*

Rayon staple fibers in the form of yarns or threads are immersed into a solution of ethylene-imine and casein in a proportion of casein to ethyleneimine of 1 in 3. The threads are centrifuged to remove excess liquid and immersed into a solution of phenylisocyanate in cyclohexanol. The threads are again centrifuged and inserted into a drying apparatus at a temperature of 80° C. for an hour. The fibers thus obtained may be dyed in one bath together with wool fibers without any difference in the absorption of dyestuff from the bath being noticeable between the two kinds of fibers.

40. We claim:

1. A process of producing films, fibers, foils, ribbons and the like materials capable of being dyed by acid wool dyestuffs, which process comprises impregnating a textile material having per se insufficient affinity for acid dyes with a solution of a resinous composition comprising an alkylene imine, a protein and a member selected

from the class consisting of arylisocyanates and arylisothiocyanates and heating the impregnated fibers until they are completely dry, whereby joint polymerization of the constituents with formation of a resin occurs.

5

2. A process of producing fibers, films, foils, ribbons and the like materials capable of being dyed by acid wool dyestuffs which process comprises impregnating a textile material having per se insufficient affinity for acid dyes with a solution of a mixture of a protein and an alkylene imine, immersing the impregnated textile materials into the solution of a member selected from the class consisting of arylisocyanate and arylisothiocyanates and heating said textile materials to a temperature sufficiently elevated to cause joint polymerization of the constituents with formation of a resin.

10

3. A process of producing fibers, films, foils, ribbons and the like materials capable of being dyed by acid wool dyestuffs which process comprises impregnating a textile material having per se insufficient affinity for acid dyes with a solution of ethyleneimine and casein, immersing the impregnated textile materials into a solution of phenylisocyanate and heating the textile materials to a temperature of from 60 to 100° C. until said textile materials are completely dried, whereby joint polymerization of the constituents with formation of a resin occurs.

15

4. Textile materials impregnated with a resin being the product of a joint polymerization of one alkylene imine, a protein and a compound selected from the class consisting of arylisocyanates and arylisothiocyanates, which resin is substantially insoluble in acids and alkalies and imparts to said textile materials affinity for acid dyes.

20

5. Textile materials impregnated with the resin produced by jointly polymerizing ethylene imine, casein, and phenylisocyanate, which resin is substantially insoluble in acids and alkalies and imparts to said textile materials affinity for acid dyes.

25

PAUL ESSELMANN.

JOSEF DÜSING.

30

40

45